

G. MOJANA.

PROCESS FOR TREATING ZINKIFEROUS SUBSTANCES.  
APPLICATION FILED DEC. 14, 1906.

961,514.

Patented June 14, 1910.



WITNESSES:

W. M. Avery

J. P. Davis

INVENTOR

Guido Mojana

BY

Munro Co

ATTORNEYS

# UNITED STATES PATENT OFFICE.

GUIDO MOJANA, OF MILAN, ITALY.

## PROCESS FOR TREATING ZINKIFEROUS SUBSTANCES.

Specification of Letters Patent. Patented June 14, 1910.

961,514.

Application filed December 14, 1906. Serial No. 347,846.

To all whom it may concern:

Be it known that I, GUIDO MOJANA, civil engineer, subject of the King of Italy, residing at Milan, Italy, have invented new and useful Improvements in Processes for Treating Zinkiferous Substances, of which the following is a specification.

My present invention relates to a process for treating calamin smithsonite, blonde, concentrates and tailings, zinc ashes, namely the residues of the zinc plating industry and all other industries where zinc is treated, with the object of forming a soluble compound with the zinc contained in such materials; such compound is then extracted from the remainder of the mass by lixiviation, depurated and eventually electrolyzed in order to obtain metallic zinc.

It is well known that when calamin, for instance, is treated with chlorin in various conditions of temperature and pressure only a part of the zinc it contains is transformed into chlorid. The same happens with all the ores and materials containing zinc not in the state of sulfid. If the zinc is contained in the form of sulfid, as in the blonde, by operating under certain conditions upon the molten mass, the chlorin is rapidly absorbed, sulfur is set free and a chlorid of zinc is formed. The Ashcroft and Swinburn process is based upon this reaction and cannot be applied to other ores than blonde nor to roasted blonde, nor to ashes.

I have discovered that by acting in the presence of porous carbon and under certain determined conditions the zinc contained in the calamin can also be almost totally transformed into a soluble compound (chlorid) and the same result is obtained with the other zinkiferous substances. The process based upon said discovery may thus also be applied to calcined and uncalcined calamin, blonde smithsonite, zinc ashes, concentrates and tailings. For this purpose I may use charcoal, or coke obtained from the distillation of coal, peat, lignite, and wood, and which is broken into small particles. It must be intimately mixed with the zinkiferous substances and preferably wetted a little before mixing the temperature must generally be above 75° centigrade; chlorin is at first absorbed in considerable quantity the absorption then grows less rapid and becomes very slow. During the operation carbonic acid, oxid of carbon and naturally the chlorin not absorbed are given off from the

mass. For this reason the apparatus for working the process has been so designed as to compel the gases given off from the mass which has been almost completely treated to pass through another mass only slightly treated. Chlorin is thus all absorbed and the gases are set free in the atmosphere.

According to circumstances it is well to inject together with the chlorin (but only at intervals) a jet of steam.

The reaction between gaseous chlorin and the zinc ores is likely to take place in consequence of the presence of steam, developing either from the humidity, natural or artificial, of the ore under treatment, or from the humidity the chlorin carries.

The quantity of water required for the reaction is small in comparison with the amount, which would correspond with the quantity of chlorin, as reckoned on the base of the chemical equations, this depending upon the circumstance that water is being produced in the same quantity as required by the reaction which is going on.

The reaction may be considered as consisting of two phases, respectively represented by the equations:



As the chlorid of zinc thus formed is a strongly hygroscopic substance which absorbs water even at temperature of about 200° C., it may happen that, while the chlorination is going on and the amount of chlorid of zinc is increasing, the steam, necessary for the completion of the reaction may not be present in the parts of the apparatus situated at a distance from the point of entrance of chlorin. In this case the introduction of a special jet of steam may prove advantageous.

Other elements by which the reaction is influenced are, besides the presence of steam, the temperature, the quantity of carbon and its intimate mixture with the ore.

By the use of the comminuted carbon the reactions, by which the chlorid of zinc is formed from the charge, are obtained at a comparatively low temperature, the reactions taking place at about 100° C., though the best results are obtained at about 200° C.

In the annexed drawing I have illustrated two different forms of construction of the apparatus, which may be used for carrying out my process.

Figure 1 is a vertical section of a continuous action apparatus. Fig. 2 is a plan view of a modified form, Fig. 3 is an elevation, Fig. 4 a section on line A—B of Fig. 3, and Fig. 5 a section on line p—q of Figs. 3 and 4, of an alternating action apparatus.

The continuous apparatus shown in Fig. 1 consists of a cylinder S made in one piece or formed of special bricks and mortar that 10 resist the action of chlorin, the cylinder being as thin as possible. The pipe t in the lower part serves for introducing chlorin. The heating of the cylindrical retort is attained by circulating around and inside 15 same the products of combustion of a common furnace properly diluted with air. The hot gases enter the earthenware pipe L, with thin walls located inside the retort S, and rise through it, then they come down into 20 the annular chamber C' along the retort and again rise along C<sup>2</sup>, whence they pass into an iron pipe which discharges them into the atmosphere. In the bottom of the retort there is a door for the discharge, the 25 charging being effected from the top.

The alternating action apparatus (Figs. 2 to 5) consists of two retorts 1, 2 (Fig. 3), arranged in series. These retorts are each surrounded by two annular chambers C', C<sup>2</sup> 30 communicating with each other at their lower portion and forming two jackets around the retort. A pipe M connects with the upper part of the annular chamber C' and an outlet pipe leads from the upper part 35 of the chamber C<sup>2</sup>. The retorts are heated by the combustion gas from the furnace which enters through the inlet pipe M and passes downward through the annular chamber C' and then upward through the chamber C<sup>2</sup> to the outlet pipe. Chlorin is introduced so that after it has gone through the 40 retort 1 from bottom to top it passes into retort 2 through pipe u<sup>2</sup> also from bottom to top. When the retort 1 is saturated with 45 chlorin this is sent direct into retort 2 and the former is then discharged from the bottom by removing the lower cover E (kept against the bottom by a screw). When the retort 1 is recharged chlorin from retort 2 is sent 50 through it until retort 2 is saturated and so on. These operations are effected by using in addition to pipes u' and u<sup>2</sup> cocks r', r<sup>2</sup> and R this latter being a three way cock. The pipe a which supplies the chlorin can be connected by the cock R with the pipe b leading to retort 1, or with the pipe c leading to retort 2. When the pipe a is connected with pipe b, the chlorin will enter the retort 1, and as the retort 1 is then closed at the top, 55 the chlorin, not absorbed in retort 1, will pass with the other gases into the pipe u<sup>2</sup>. The cock r<sup>2</sup> in the pipe u<sup>2</sup> being open, the chlorin will pass through pipe c into the retort 2 where it will be absorbed. At this time the 60 retort 2 is open at the top so that the gases 65

will be discharged into the atmosphere. During this period the cock r' remains closed. When the charge in retort 1 is saturated, the retort is discharged and is then recharged after the cock R has been 70 turned so as to cause the pipe a to communicate with the pipe c, and the cock r<sup>2</sup> has been closed and the cock r' opened. Then retort 2 is closed at the top, retort 1 being left open at the top after the recharging. This is 75 continued until retort 2 is saturated and then the operation is repeated.

In the continuous apparatus a partial discharge is effected at regular intervals of time and it is then at once refilled from the 80 top until the retort is full.

The two apparatuses described show one of the ways of carrying out my process, but they can be modified in many ways: the retorts for instance may not be of circular 85 section, the inside earthenware pipe L in the first apparatus may be dispensed with or changed as also the circulation of the gases and so on. Where convenient the draft of the heating gas may be increased by a suc- 90 tion at the discharge of the heating chamber. The heating may also be obtained by circulating around the retort, in an annular chamber or jacket, steam at a suitable temperature and pressure or by introducing 95 steam inside the retort together with the chlorin. An important simplification can be obtained by heating the retort electrically, that is to say by passing a current of suitable voltage through an iron coil around the re- 100 tort or through a mass of granular coke around the retort, or by passing the current through the mass of coke and zinkiferous substance contained in the retort and upon which the chlorin must act. The mass which 105 has been thus treated is first sieved for the purpose of separating the charcoal from the remainder. This is taken into lixiviation tanks and treated with the washing water of said charcoal. The mixture obtained by 110 lixiviation is made hot by the introduction of a jet of steam. It is then passed through a filter press. The solid part which remains in the filter press may eventually be treated in any suitable manner to obtain silver 115 or lead, but this forms no part of the present invention. The liquid containing the chlorids of Zn, Pb, Fe and Mn. are cooled at 0° centigrade and filtered, thus separating Cl<sub>2</sub> Pb<sub>2</sub>; the liquid is then 120 successively treated with oxidants (such as chlorin, calcium hypochlorite and with substances containing oxid. of zinc (calamin, roasted blonde, calcined calamin or others) and it is then filtered. I thus get a solu- 125 tion of Cl<sub>2</sub>Zn which may at once be subjected to electrolysis. Or the said solution may be dried, and in such case the chlorid of zinc thus obtained may be placed on the market or it may be melted and in that con- 130

- dition subjected to electrolysis. When treating the solution or the molten salt by electrolysis the metallic zinc will gather on the cathode and the chlorin on the anode. This 5 chlorin is sent into the chlorinating tub after it has been dehydrated if necessary, and is then heated by passing through an earthenware coil arranged within the furnace.  $\text{Cl}_2\text{Zn}$  may also be separated from the mass 10 discharged from the charcoal, by sublimation in an earthenware retort above the boiling point of  $\text{Cl}_2\text{Zn}$ , concentrating the vapors in a suitable tank, depurating the  $\text{Cl}_2\text{Zn}$  sublimated and electrolyzing when necessary. 15 The process, when electrolysis is used, constitutes a closed cycle. In order to make up for the inevitable losses it will be necessary to furnish the cycle with a certain quantity of chlorin from one of the apparatuses 20 in use for the electrolytic production of soda. Having now fully described my said invention and how the same is to be performed, what I claim is:
1. In a process for the treatment of zinkiferous substances, subjecting the said substances to the action of chlorin in the presence of porous carbonaceous matter and moisture.
  2. In a process for the treatment of zinkiferous substances, at a comparatively low

temperature, subjecting the same to the action of chlorin in the presence of porous carbon and steam.

3. In a process for the treatment of zinkiferous substances, at a comparatively low 35 temperature, subjecting the same to the action of chlorin in the presence of porous carbon and steam, removing the carbon from the mass thus obtained, and lixiviating, filtering, and treating the liquid residuum 40 with oxidizing agents and oxid of zinc.

4. A process for the treatment of zinkiferous substances, at a comparatively low 45 temperature, consisting in subjecting the same to the action of chlorin in the presence of porous carbon and steam, removing the carbon from the mass thus obtained, lixiviating, filtering, and treating the liquid residuum with oxidizing agents and substances containing oxid of zinc, to obtain 50 zinc chlorid, and electrolyzing the zinc chlorid to obtain metallic zinc.

In testimony whereof I have signed my name to this specification in the presence of two subscribing witnesses.

GUIDO MOJANA.

Witnesses:

B. CARLO SALVOLI,  
M. SIERSDORFER.